

Sept. 9, 1930.

J. G. DONALDSON ET AL

1,775,159

METAL AND PROCESS OF MANUFACTURE

Filed Dec. 21, 1926

4 Sheets-Sheet 1



Fig. 1.

INVENTOR  
Joseph G. Donaldson  
Henry S. Cole

BY  
J. P. Edwards  
ATTORNEY

Sept. 9, 1930.

J. G. DONALDSON ET AL

1,775,159

METAL AND PROCESS OF MANUFACTURE

Filed Dec. 21, 1926

4 Sheets-Sheet 2



Fig. 2.

INVENTOR  
Joseph G. Donaldson  
Henry S. Cole  
BY  
J. W. Cullen  
ATTORNEY

Sept. 9, 1930.

J. G. DONALDSON ET AL

1,775,159

METAL AND PROCESS OF MANUFACTURE

Filed Dec. 21, 1926

4 Sheets-Sheet 3



Fig. 3.

INVENTOR  
Joseph G. Donaldson  
Henry S. Colvin  
BY  
J. E. Edmunds  
ATTORNEY

Sept. 9, 1930.

J. G. DONALDSON ET AL

1,775,159

METAL AND PROCESS OF MANUFACTURE

Filed Dec. 21, 1926

4 Sheets-Sheet 4



*Fig. 4.*



*Fig. 5.*



*Fig. 6.*

INVENTOR  
Joseph G. Donaldson  
Henry S. Cola  
BY  
J. T. Edmunds  
ATTORNEY

## UNITED STATES PATENT OFFICE

JOSEPH G. DONALDSON AND HENRY L. COLES, OF HAMILTON, OHIO, ASSIGNEES TO  
GUARDIAN METALS COMPANY, OF HAMILTON, OHIO, A CORPORATION OF DELA-  
WARE

## METAL AND PROCESS OF MANUFACTURE

Application filed December 21, 1926. Serial No. 156,107.

This invention relates to a new metal which possesses many properties and advantages that make it of distinct value in the commercial arts.

5 This new metal possesses great ductility and toughness, has higher heat conductivity and electrical conductivity than has heretofore been produced under like conditions, and at the same time is resistant to attacks made 10 by means of high heat locally applied such as the heat of the oxy-acetylene blow torch. The metal is especially resistant to attacks by a cutting torch acting in conjunction with the fluxing rod or to the oxygen lance in its various forms.

This new metal is of large crystalline structure, and its purity is of a percentage not heretofore attained.

In this invention a metal, such as copper, is 20 taken in a relatively pure condition and only a relatively small change is made in its purity, but as a result thereof there are material and marked changes in its crystalline structure and in its physical properties. That 25 is, radical changes in the crystalline structure and properties are made without a particularly marked change in chemical analysis.

The accompanying drawings illustrate portions of the invention, and the preferred 30 temperature ranges and amounts of deoxidizing agent, and further illustrate some of the examples of microphotographs of the metals.

In these drawings

Fig. 1 is a chart illustrating the preferred 35 amount of deoxidizing agent to be included at particular temperatures for pouring;

Fig. 2 represents a preferred cooling curve for obtaining the desired results described herein;

40 Fig. 3 illustrates cooling curves of metals in which various elements have been added; and

Figs. 4, 5, and 6 are reproductions of microphotographs of various examples of the 45 metals.

These marked changes in structure and properties are accomplished, in the manner we prefer, by submitting a metal to a definite process of deoxidization, then deliberately adding nuclei forming substances, and then

cooling in a definite manner. If desired, the cooling may be varied and the resulting metal subjected to a definite method of heat treatment.

The results of such manufacture give a new 55 metal possessing the advantageous characteristics above presented, and the crystalline structure of the metal shows large crystals with definite boundaries, while frequently and in the majority of cases there is found 60 in the boundaries more or less quantity of a material appearing dark and amorphous.

The chemical composition of this amorphous material has not been determined.

From experiments and use, this new metal 65 having large grain size cannot be cut with an acetylene blow torch, and if of sufficient size cannot be melted by large blow torches; and it offers exceptionally high resistance to the fluxing action of molten iron when attacked by the cutting torch acting in conjunction with the fluxing rod; or when attacked by the oxygen lance. The amorphous material, particularly, resists the attacks of 70 these destructive devices.

The general process for manufacturing this new metal may be considered as above outlined, but there are, however, certain precautions which should be noted in order that the most efficient results may be obtained. 75 One of these precautions is to thoroughly mix or stir into the molten metal the deoxidizing agent so that it is thoroughly distributed throughout all of the metal. Thorough stirring is also desired when the 80 nuclei forming substances are added. In addition, it has been found advantageous to cover the molten mass with a material which prevents the oxidization of the surface metal.

This covering has been found of advantage during the heating step, during the deoxidization step, during the step of distribution of the nuclei forming material, and during the cooling step of the process. It has been found that the heat conductivity and the electrical conductivity of the resulting metal increases in a ratio with the amount of reduction of the oxides in the metal. Therefore, it has been found advisable to keep the oxygen, iron and impurities as low as possible. When these 85

conditions are true the crystals of the resulting metal are of large size and there is a definite grain boundary between them. With the addition of the nuclei forming material 5 it has been found that in the majority of cases an amorphous material is deposited in the grain boundaries and is readily discernible under the microscope. It has also been found that certain materials act as deoxidizers and at the same time act as nuclei forming substances. Carbon in the form of graphite gives such a double satisfactory action.

In producing this new metal it is preferred 15 to choose a metal of high conductivity, such as copper and to bring this metal to a molten condition. In practice this is preferably accomplished by using a furnace of the direct arc type, or a rotating furnace of the indirect 20 arc type.

After the metal has been made molten it is essential that the same be brought to a high degree of deoxidization. The best results have been obtained when the deoxidization 25 has been particularly high. Any suitable deoxidizing agent may be employed and it is particularly desirable in order to obtain ideal results to use that deoxidizer which will remove the oxides from the 30 metal and will least alloy therewith. We have found that 20% of commercial cupro silicon is advantageous for this purpose when copper is used as a base metal. We have also found that carbon, preferably in the form 35 of powdered graphite, is most excellently suited for the deoxidization of certain metals, especially such a metal as copper. In the last instance, carbon unites with the oxygen and forms a gas (carbon monoxide or carbon dioxide) and if the metal is properly stirred 40 the gas will escape from the mixture. The carbon in the form of graphite also performs another function as will be set forth below in detail.

45 If an excess of certain deoxidizers is used, an alloy will be formed between the deoxidizing agent and the metal, with the result that the conductivity of the metal will be lowered, and its resistance to heat attack locally applied consequently greatly impaired.

Our experiments have shown that there is a direct relation between the heat of the metal and the amount of the deoxidizing agent which must be used. Reference is, therefore, 55 made to Fig. 1 in which a working curve is reproduced to determine the amount of the deoxidizing agent to be used to give the best results when the molten material is copper at a definite temperature. For instance, if 60 the temperature of the molten copper metal is 2300° F., the quantity of the deoxidizing agent will be .70%. Again, if the temperature of the molten material is 2450° F., the quantity of the deoxidizing agent will be 65 .35% as will be noted from the curve. In

carrying out the addition of the proper amount of deoxidizer, it is assumed that a charge of 5000 lbs. is introduced into the furnace and that it has been brought to a temperature of 2300° F., then the requirement 70 of the deoxidizer of the .70% is added. We now assume that the deoxidizing agent is cupro silicon and that it is of the trade purity considered as being 20%. We find that  $5000 \times .0070 = 35$ , which means that 35 lbs. of 75 20% cupro silicon is to be added when the temperature of the mass is at 2300° F. This gives a sufficient quantity of the deoxidizer 80 that will perform its function of deoxidization without alloying with the metal to a detrimental extent. As a result of this example, we find that the copper plate or casting obtained, has a purity of 99.97%. When other deoxidizing agents are employed a curve similar to the one shown in Fig. 1 may 85 be prepared. It has been found that the original copper (commercial copper) employed has a purity of about 99.90% and that during the treatment, or manufacturing, the 90 purity reduces to about 99.50 due to some absorption of oxygen and of impurities from the furnace lining. Before the completion of our improved process this is raised so that the final result has the purity above mentioned, i. e., 99.97% or better.

The curve shown in Fig. 1 also shows the temperature at which the metal should be poured. Some of the best results, however, follow when the metal is poured at or above the temperature of 2270° F.

After the metal has been deoxidized there is added a small proportion of certain materials or substances, preferably in powdered form, which materials are intended to serve as a nuclei for the formation of large crystals in the metal. Preferably there is added 1/8 of 1% to 1/4 of 1% of these materials or substances and the metal is preferably stirred in order to thoroughly mix these substances into the mass. This step is of importance as it has a bearing on the fineness or purity of the final metal.

The mixing in an electrical furnace of the rotating type has been found most excellent. Several different substances have been employed as the nuclei forming material. In one instance we have found that good results may be obtained by using aluminum magnesium silicates such as mica or alberene stone. Excellent results followed the use of zirconium silicate, ( $ZrSiO_4$ ), barium sulphate ( $BaSO_4$ ), sodium aluminate ( $Na_2AlO_4$ ), molybdenum sulphide ( $MoS_2$ ), vanadium pentoxide ( $V_2O_5$ ), and graphite. These substances, themselves, it will be noted, are relatively insoluble in molten steel, and when they are combined with the deoxidized base metal, as herein described, produce the advantageous new metal which resists the action of the oxygen lance.

70

75

80

90

95

100

105

110

115

120

125

130

After the nuclei forming substances have been added and thoroughly mixed the resulting molten metal is poured into suitable molds. Preferably the pouring is made when the temperature of the mass is about 2270° F. The metal in the molds is allowed to cool very slowly. Care should be taken to cover the metal with a suitable non-conducting substance after pouring, especially if the casting is small. The cooling is an important step in the preparation of this metal, as above noted, for the purpose of permitting the formation of the large size grain crystals. It is preferred to cool at a predetermined rate in order that the cooling may be satisfactorily accomplished.

Reference is now made to Fig. 2 of the drawings in which there is shown a cooling curve that permits the formation of the desired crystalline structure. It will be noted that in this curve the approximate point of freezing of the metal is pointed out, and the various changes in the curve show approximate temperatures where there are various changes being made in the crystalline structure during the cooling.

It has been found that the best results are obtained when there is special controlling of the cooling until the temperature reaches about 1300° F. The cooling from 1300° F. to 700° F. is not quite so important, but should be controlled as to the rate of cooling. Below 700° F. the rate of cooling may be rapid.

If the casting cools too quickly or in such a manner as not to give a satisfactory result it may be subsequently heat treated and the recooling controlled in accordance with the curve in Fig. 2 of the drawings.

In the case of such subsequent heat treatment, the casting should be brought to a temperature of approximately 1900° F. and held at that point until such time as the whole casting has been raised to this temperature. It should then be allowed to cool very slowly until the temperature reaches about 700° F. and from this point down it may be allowed to cool quickly if desired.

When certain materials in a pulverulent condition are added to the metal in molten condition and thoroughly stirred therewith it has been found that the cooling curve of the metal will rise after the same has solidified. This rise in temperature usually indicates a crystalline change. Such crystalline changes are shown in Fig. 3 of the drawings where curve 1 shows the cooling curve of a metal which has been deoxidized by cupro silicon and has had added to it alberene stone or the like as the nuclei forming substance. Curve 2 shown in Fig. 3, illustrates the cooling curve of a metal which has been deoxidized with the cupro silicon and which has had graphite added to it as the nuclei forming substance.

Examination of this new metal under the microscope will show a peculiar and characteristic crystalline structure. This structure shows large grains and a deposit of a dark material in the grain boundaries.

In disclosing the advantages of the process herein set forth there is illustrated in Figs. 4, 5 and 6 of the drawings diagrammatic representations of microscopic pictures of various samples of metal. In Fig. 4 there is illustrated the ordinary cast copper having therein no nuclei forming substance such as alberene stone or graphite and there is in that illustration evidence of solid solution (alloying) as shown by mixed crystals appearing in the metal. It will be noted that there are a large number of relatively small size crystals such as 3, 4 and 5 and the like.

The representation shown in Fig. 5 is a magnified view of cast copper made in accordance with this process wherein alberene stone or the like was used as the added material for nuclei forming purposes. In that figure it will be seen that there are large grain crystals, portions thereof being illustrated at 6, 7 and 8. It will be noted that the grain boundaries are very clearly defined and that there is shown in the boundaries the amorphous material 9 which varies in size and, therefore, amount. It will therefore be noted that the amorphous material throughout the grain boundaries creates an envelope around each grain. This is the material which is especially resistant to an attack by local high heat. In Fig. 6 there is shown a crystalline structure of cast copper made in accordance with the process herein where the nuclei forming material is graphite. In this instance also there is noted the large grain crystals 10, 11, 12 and 13 while the boundaries between the crystals are clearly defined and the amorphous material 14 is present.

For the purpose of comparison the reproduction in Figs. 4, 5 and 6 are taken from photo micrographs of the same degree of magnification, i. e. 150 magnification.

The new metal herein disclosed is a material improvement on the metal disclosed in our copending application, alloys and material employing the same, filed May 19, 1923, Serial No. 640,226, and the divisional application therefrom, refractory materials and process of producing the same, filed January 16, 1925, Serial No. 2,863. In the present process and product there is added a nuclei forming substance. This is not true of the process and product set forth and claimed in our copending applications, and also there is a smaller amount of cupro silicon employed in the present process. In the process described in the copending applications there is an alloying of the material which alloying reduces the heat conductivity of the resulting metal. This feature is particularly undesirable in the present process for the present

product is substantially free of oxides and other impurities. Another distinction of the present product from that of the product in the copending applications is that the present product is of a fewer number of large size grain crystals while the former product is made up of a large number of small size crystals. In the copending applications by reason of the small amount of carbon there is considerable oxide in the resulting metal, while in the present metal by using a different amount of carbon the oxide becomes reduced so that a substantially pure unalloyed copper is obtained and consequently a materially larger grain structure, which is of advantage in increasing the heat conductivity and the electrical conductivity as well as the resistance to the blow torch and the oxygen lance.

It will, therefore, be seen from the above description that the new metal has many advantages and properties over like metal of less purity, and that this new metal is of particular advantage as being resistant to local high heat as applied by the oxygen lance and by the burning of molten iron or molten iron oxide thereagainst. Likewise, there is a material improvement in the property of heat conductivity and electrical conductivity of the new metal over the metal before being subjected to this process. All of these features are of very material advantage in the manufacture of metals and plates formed thereof, and which are exceptionally desirable in producing vaults and safes. In addition, there is also a special advantage of the new metal with its high electrical conductivity for it may be used for power transmission lines and the like to a material advantage and saving.

We claim:

1. A process of forming a new metal which consists in raising a base metal to a molten condition, deoxidizing said metal, adding a substance relatively insoluble in molten steel, and cooling in a manner to cause the substance to be deposited in the amorphous material in the grain boundaries of the crystals.

2. A process of forming a new metal which consists in raising a base metal to a molten condition, deoxidizing said metal, adding  $\frac{1}{8}$  of 1% to  $\frac{1}{4}$  of 1% of alberene stone, and cooling in a manner to cause the said alberene stone to be deposited in the amorphous material in the grain boundaries of the crystals, said cooling being carried on at a predetermined rate that permits the formation of crystalline structure with the majority of crystals of relatively large size.

3. A process of forming a new metal which consists in raising a metal of high conductivity to molten condition, adding a sufficient quantity of material that will deoxidize said metal without leaving an excess to alloy

therewith, adding a nuclei forming substance, and cooling in a manner to permit the formation of large crystals and the deposit of said nuclei forming substance in the amorphous material of the grain boundaries. 70

4. A process of forming a new metal which consists in raising commercial copper to a molten condition, deoxidizing said copper, adding nuclei forming substances, and cooling at a rate that gives a crystalline structure with the majority of crystals of relatively large size and the deposit of said nuclei forming substance in the amorphous material of the grain boundaries. 75

5. In the process of treating copper, the 80 step of adding  $\frac{1}{8}$  of 1% to  $\frac{1}{4}$  of 1% of nuclei forming substances.

6. The process of forming a new metal which consists in raising commercial copper to a molten condition, deoxidizing said copper, adding  $\frac{1}{8}$  of 1% to  $\frac{1}{4}$  of 1% of nuclei forming substances, and cooling in a manner to permit the formation of large crystals and the deposit of said nuclei forming substance in the amorphous material of the 90 grain boundaries. 85

7. In the process of treating commercial copper to improve its purity and crystalline structure, the steps of raising the copper to a molten condition, adding a deoxidizing 95 agent, the amount of which is dependent upon the temperature of the copper, adding a nuclei forming substance, and cooling whereby the said nuclei forming substance deposits in the amorphous material of the grain 100 boundaries.

8. The process of increasing the purity and grain structure of copper, which consists in raising the copper to a molten condition, adding commercial cupro silicon to deoxidize 105 said copper, the amount of said cupro silicon being dependent upon the temperature of the molten copper at the time of adding said cupro silicon, adding  $\frac{1}{8}$  of 1% to  $\frac{1}{4}$  of 1% of nuclei forming substances, and cooling in 110 a manner to permit the formation of large crystals and the deposit of said nuclei forming substance in the amorphous material of the grain boundaries.

9. The process of increasing the purity and 115 resistance to local high heat of copper, which consists in melting copper in an electric furnace, covering the surface thereof with powdered charcoal to prevent oxidization, adding a predetermined amount of 20% cupro silicon to deoxidize said copper without alloying therewith, the amount of said cupro silicon being governed by the temperature of said copper at the time of adding the same, stirring, adding a nuclei forming material 120 in the quantity of  $\frac{1}{8}$  of 1% to  $\frac{1}{4}$  of 1%, pouring said material at a temperature above 2270° F., covering the copper after pouring with non-conductive substances, and cooling 125 slowly to permit the formation of large crys- 130

5 tals and permit the deposit of said nuclei forming substance in the amorphous matter of the grain boundaries.

10. A metal of high conductivity which has been deoxidized by 20% cupro silicon and which has large grain size and has an aluminum magnesium silicate deposited in the amorphous material in the grain boundaries.

11. Cast copper plate having large crystalline structure and which has been deoxidized by employing a predetermined amount of 20% cupro silicon and which has had added thereto from  $\frac{1}{8}$  of 1% to  $\frac{1}{4}$  of 1% 15 alberene stone.

12. An article of manufacture being copper with substantially all the oxides removed, said article having relatively large crystals and having a substance relatively insoluble 20 in molten steel deposited in the amorphous material in the grain boundaries.

This specification signed this 14th day of December, 1926.

JOSEPH G. DONALDSON.  
HENRY L. COLES.

25

30

40

45

50